# EUROPEAN PATENT SPECIFICATION

(11) **EP 0 286 318 B1**
(45) Date of publication and mention of the grant of the patent: **24.05.1995**
(21) Application number: 88302889.6
(22) Date of filing: 30.03.1988
(51) Int. Cl.: D21F 11/00, D21H 21/06

(54) **Maufacture of wet laid nonwoven webs**
Herstellung von nassgelegten, nichtgewebten Faserbahnen
Fabrication de bandes fibreuses non tissées par voie humide

(30) Priority: 06.04.1987 US 35059
(43) Date of publication of application: 12.10.1988
(73) Proprietor: JAMES RIVER CORPORATION, Norwalk Connecticut 06856 (US)
(72) Inventor: Tse, Stephen H., Richmond Virginia 23217 (US); Hollenberg, David H., Neenah Wisconsin 54956 (US); Martin, Richard L., Neenah Wisconsin 54956 (US); Manning, James H., Neenah Wisconsin 54956 (US)
(74) Representative: Archer, Philip Bruce

(56) References cited:
- GB-A- 1 049 675
- GB-A- 2 068 034
- US-A- 3 325 345

## Description

This invention relates to an improved method for the manufacture of a uniform fibrous web comprising textile length fibers by wet forming the web on a conventional paper-making machine. In one of its more specific aspects, this invention relates to a method for forming a uniform web from an unfoamed dispersion of staple length natural or synthetic fibers in water containing a small amount of an associative thickener. In one of its still more specific aspects, this invention relates to the use of a nonionic associative thickener consisting essentially of an ethylene oxide based urethane block copolymer having alternating blocks of polyethylene glycol and polyurethane as dispersant and thickener in water as the carrier for natural and synthetic fibers. In still another of its more specific aspects, this invention relates to the use of a nonionic associative thickener consisting essentially of a hydroxyethyl cellulose having a long aliphatic side chain as the dispersant and thickener for natural and synthetic cellulose fibers in a water carrier.

Methods for forming non-woven fibrous webs containing textile length fibers, e.g. synthetic fibers having a length to diameter ratio in the range of from about 300 to about 3000, in a wet paper-making process are known in the art. Generally, a viscous aqueous carrier comprising a dispersant and thickener is required for good dispersion of long thin flexible synthetic fibers, e.g. 1.5 denier by 19mm (¾ inch) fibers. The long thin synthetic fibers tend to tangle and form flocs or nits in the finished non-woven fabric formed from an aqueous dispersion suitable for wet-laying paper-making fibers on a paper-making machine.

Foam furnishes have been proposed as a viscous aqueous carrier medium to ensure good dispersion of the long fibers, for example, as disclosed in U.S. Patent No.4,049,491. While aqueous foams have been shown to be suitable carriers for staple length fibers, the high viscosity of foam results in relatively slow drainage of water from the dire of the paper-making machine. Other methods proposed for this purpose include the addition of thickeners to an unfoamed water carrier, for example, as disclosed in U.S. Patent No.3,098,786 wherein deacetylated karaya gum and sulphuric acid are included in the water-fiber furnish, and in U.S. Patent No.3,013,936 in which a synthetic fiber is modified to include available hydrophilic groups and the thickener is a water-swellable, water insoluble gum. Various water soluble polymers are disclosed as dispersing aids for staple length fibers in U.S. Patent Nos.3,808,095 and 3,794,557 including anionic, cationic and nonionic dispersing agents, among which is polyethyleneoxide.

There is disclosed in GB-A-1 049 675 a process of making fibrous webs in which there is proposed the use of hydroxyethylcellulose in order to increase the viscosity of the water of the aqueous suspension.

There is disclosed in the US-A-3 325 345 a process of forming water-laid products from cellulosic pulp containing polymeric thermoplastic particles. Examples of the preferred polymers are hydrophobic polymers such as those derived from olefinic hydrocarbons such as polymers and copolymers of ethylene, propylene etc.

According to the invention there is provided a method for the preparation of a fibrous web comprising textile length fibers, as defined in the accompanying claims.

There is described below an improved method for forming fibrous webs from a water furnish containing textile length fibers which comprises the inclusion of an associative thickener in the water making up the fiber furnish. Associative thickeners have been developed primarily for use in the formulation of latex paints. The urethane block copolymers are described by E.J. Schaller and P.J. Rogers-Moses, Resin Review, Vol. XXXVI, No.2, pp 19-26, incorporated herein by reference. The hydrophobically-modified hydroxyethylcellulose nonionic associative thickeners are described by K.G. Shaw and D.P. Liepold, Journal of Coatings Technology 57, No. 727, pp 63-72 (August, 1985). In latex paints, associative thickeners are used to give the formulation certain desirable properties e.g., enough viscosity to resist running and over-spreading; spatter resistance; and improved levelling properties. We are not aware of any prior art in which these associative thickeners have been used in the manufacture of a water laid fibrous web.

In the process of this invention, a dispersion of fibers in water is made up with a small amount of an associative thickener which acts as both a surfactant (or dispersant) and as a thickener, slightly increasing the viscosity of the water carrier medium and acting as a lubricant for the fibers. One class of nonionic associative thickeners Preferred in the process of this invention comprises relatively low (10,000 to 200,000) molecular weight ethylene oxide based urethane block copolymers and is disclosed in U.S. Patent Nos.4,079,028 and 4,155,892. These associative thickeners are particularly effective when the fiber furnish contains 10% or more staple length hydrophobic fibers. Commercial formulations of these copolymers are sold by Rohm and Haas, Philadelphia, PA, under the trade names Acrysol RM-825 and Acrysol Rheology Modifier QR-708. Acrysol RM-825 is a 25% solids grade of polymer in a mixture of 25% butyl carbitol (a diethylene glycol monobutyl ether) and 75% water. Acrysol Rheology Modifier QR-708, a 35% solids grade in a mixture of 60% propylene glycol and 40% water, has been found to produce excellent results in test runs as reported in Examples I and 2, below.

Another class of associative thickeners, preferred for making up fiber furnishes containing predominantly cellulosic fibers, e.g. rayon fibers or a blend of wood fibers and synthetic cellulosic fibers, such as rayon, comprises modified nonionic cellulose ethers of the type disclosed in U.S. Patent No.4,228,277, and sold under the trade name Aqualon by Hercules Incorporated, Wilmington, Delaware. Aqualon WSP M-1017, a hydroxyethyl cellulose modified with a C₁₀ to C₂₄ side chain alkyl group and having a molecular weight in the range of 50,000 to 400,000 was found to be particularly effective for the preparation of fiber furnishes comprising rayon fibers, as illustrated in Example 3.

We have found that the urethane block copolymers described hereinabove are effective as a thickener and dispersant for the preparation of fiber furnishes containing textile length hydrophobic fibers, for example, polyester, acrylic, polyamide, polyolefin, and modified acrylic fibers in a water carrier. The nonionic urethane block copolymers are of especial importance in the preparation of unfoamed fiber-in-water furnishes containing textile length hydrophobic fibers alone or in admixture with cellulosic paper-making fibers. The modified nonionic cellulose ethers described hereinabove are particularly useful in the preparation of fiber furnishes in which the textile length fibres are cellulosic fibers, e.g. rayon fibers, alone or in admixture with natural wood fibers and similar cellulosic fibers suitable for use in making paper. Although conventional paper-making fibers are preferred in such mixtures, high bulking fibers which have been subjected to chemical or mechanical treatment, e.g. caustic treatment or high energy wet or dry milling, to kink and curl the fibers may be included in the furnish.

The hydrophobic fibers forming the aqueous dispersion and the ultimate fabric may comprise from about 10 to 100% by weight of staple length fibers and from 0 to 90% conventional wood fibers. Synthetic fibers in the size range of 1 to 4 denier by 19 to 38mm (¾ to 1.5 inch) are preferred. Suitable textile fibers include polyester fibers, e.g. those sold under the trade names Trevira, Dacron, Kodel, Fortrel, etc.; acrylic fibers, e.g. those sold under the trade names Creslan, Acrilan, Orlon, etc. polyamide fibers, e.g. nylons; polyolefin fibers, e.g. polypropylene; and modified acrylic fibers including those sold under the trade name Dynel. Inorganic fibers, including glass fibers may comprise part or all of the textile length fibers. Any of the wood cellulose fibers may be used with either type nonionic associative thickener; those comprising or consisting essentially of soft wood fibers are preferred. Other fibers may be used in conjunction with or instead of wood cellulose fibers. In addition to rayon, other known cellulosic fibers, e.g. cotton linters, may be used in the process. The modified nonionic hydroxyethyl cellulose associative thickeners are, however, relatively ineffective for dispersion of hydrophobic fibers.

For best results, the wood cellulose pulp is dispersed in water prior to adding the associative thickener, followed by the addition of the associative thickener and then the addition and dispersion of the staple length fibers. Finally, the dispersion of mixed fibers in an unfoamed water carrier is diluted to the desired headbox consistency and dispensed onto the forming wire of a conventional paper-making machine. An anti-foam agent may be added to the dispersion to prevent foaming, if necessary, and a wetting agent may be employed to assist in wetting the staple length fibers if desired.

The fibers preferably are made up into an aqueous dispersion suitable for wet forming on a moving wire former in the following manner. The wood pulp is first dispersed in water or in recycled white water to a consistency of about 1 to 2%. Then a nonionic associative thickener is added to the resulting slurry in an amount within the range of about 100 to 500 ppm followed by the addition of the textile length fibers with continuous mixing under low shear conditions.

After the fibers are thoroughly blended, the slurry is further diluted with fresh water and white water to the final headbox furnish consistency, perferably to a consistency in the range of 0.05 to 0.5%, and supplied to the headbox of a paper-making machine. A non-woven fabric web may be formed from a staple length textile fiber furnish on high speed conventional Fourdrinier paper-making machines to produce a strong, uniform product of excellent formation.

In making up the fiber dispersion containing the staple length fibers, low shear agitation, as provided by a non-stapling agitator is preferred to avoid tangling of the long fibers. As illustrated in Example 2, a small amount of a conventional polymer thickener may be added to the dispersion to more precisely control drainage of white water from the wire during web formation. While a number of nonionic polymers may be used for this purpose, the anionic polymer sold under the trade name Hydraid 7300-C by Calgon Inc., Pittsburgh, Pennsylvania is particularly effective at concentrations of the order of 100 ppm. A defoamer, e.g. the product sold under the trade name DF-122 by Diamond Shamrock Company may be added, if required, during the preparation of the fiber furnish to eliminate foam formation in the dispersion.

A number of advantages result from dispersion of staple length fibers in a water solution of a nonionic associative thickener as compared with dispersions in foam or water containing surfactants and conventional polymer thickeners. The lower nascent viscosity of the aqueous carrier composition of this invention, as compared with prior art processes employing conventional thickeners or surfactants, results in higher drainage rates through the forming wire and permits formation on conventional Fourdrinier machines at high wire speeds. In contrast to prior art processes, special machines with sloping wires and conforming headboxes are not required for operation of our process. The dispersion is neither excessively thickened nor foamed, making it possible to handle the dispersion with conventional contrifugal pumps and to use conventional headboxes and forming wires, and to operate such equipment at high wire speeds. Good dispersion of the fibres is obtained without the need for high energy pulping equipment. Additionally, the total chemical usage is lower in the process of this invention than for processes currently used for forming non-woven fabric webs from staple length fibers.

The following examples further describe and illustrate the process of this invention.

### EXAMPLE 1

A batch fiber-water dispersion was made up with 2722kg (6000 pounds) of water in a mix tank equipped with a non-stapling agitator by adding in the following order:
a) 20.86kg (46 pounds) of West Coast bleached softwood slush pulp at 36% solids;
b) 726g (1.6 pounds) of nonionic associative thickener, Acrysol QR-708, 34% active (Rohm and Haas Philadelphia, PA); and
c) 7.48kg (16.5 pounds) of polyester staple, 1.5 denier x 19mm (¾ -inch) of Hoechst Trevira (trade mark) Type 101 SD OW. The mixture was agitated for 20 minutes and then pumped with a centrifugal pump to the exit side of a fan pump where it was diluted to 0.08% consistency with white water at 37.8°C (100°F) containing 82 ppm Acrysol QR-708 and 3 ppm Foammaster Defoamer DF-122 (a product of Diamond Shamrock). The nascent viscosity of the water in the mix chest and of the white water was 1.2 x 10-³Ns/m² (1.2 centipoise). The dispersion was formed on an inclined wire former producing a non-woven web with good formation. Physical properties of the product web are shown in Table II below.

### EXAMPLE II

A trial run was made with a furnish of 60 wt.% of Marathon Northern Softwood blended kraft pulp and 40 wt.% 1.5 denier x 19mm (¾-inch) polyester fibers. A 15.14m³ (4000 gallons) capacity hi-lo pulper was used to break up dried sheets of the bleached kraft pulp. 11.36m³ (3000 gallons) of fresh water heated to 31°C (88°F) was added first, then 136 kg (300 pounds) of the pulp was added. The pulp was dispersed by using both high and low agitators for 25 minutes. Then 9.07kg (20 pounds) of Acrysol QR-708 (34% active) was dissolved in 18.93 x 10-³m³ (5000 gallons) of water at 71°C (160°F) and added to the pulper followed by the addition of 0.530 m³ (140 gallons) of Calgon's Hydraid 7300-C made to 0.58 volume percent solution in water at 21°C (70°F). Then 90.7kg (200 pounds) of Heochst Trevira polyester of 1.5 denier x 19mm (¾-inch) was added while only the lower agitator mixed the stock. Since some foam appeared, 0.47 litres (one pint) of Diamond Shamrock's Defoamer DF-122 was added and the entire mix pulped for 20 minutes. It was then pumped with a centrifugal pump to a mix chest where it was diluted with another 15.14m³ (4000 gallons) of fresh water at 31°C (88°F). The mix from the mix chest was then pumped with a centrifugal pump to the machine chest without further dilution. The dispersion from the machine chest was pumped to the headbox of a wire former with a centrifugal pump where it was diluted to 0.065% consistency with white water which contained 100 ppm Acrysol QR-708 and 100 ppm Hydraid 7300-C. Table I lists the viscosity data obtained during the trial using the UL attachment to a Brookfield viscometer and Table II, below, lists the physical properties of the product web.

**TABLE I**

| Nascent Viscosity of Water Carrier | | |
|---|---|---|
| Location and Description | Viscometer Temp. °C(°F) | Viscosity cp(1 x 10-³Ns/m²) |
| Pulper - water only | 16.7(62) | 1.20 |
| Pulper - QR-708 200 ppm | 17.2 (63) | 1.21 |
| Pulper QR-708 (200 ppm) and 7300-C (200 ppm) | 16.7(62) | 2.54 |
| Machine chest QR-708 (100 ppm) 7300-C (100 ppm) | 16.7(62) | 1.49 |
| Headbox QR-708 (100 ppm) 7300-C (100 ppm) | 17.2(63) | 1.38(1) |

| | | |
|---|---|---|
| (1) The headbox viscosity was lower than the machine chest viscosity because of dilution of the stock to the headbox with plain water. | | |

### EXAMPLE 3

Approximately fifty 30 lb/rm handsheets consisting of 70% 1.5 denier x 12mm(½ inch) rayon fibers and 30% Ontario soft wood kraft pulp were made on an M/K Systems, Inc. Series 8000 Computerized Sheet Former consisting of three main components: the Sheet Former itself with its Forming and Pressing/Drying sections, a 200-litre stock tank, and a Hewlett Packard HP-85 desk top computer which controls the operation of the Sheet Former.

In the valley beater, 269 grams of wet wood pulp was mixed with 23 litres of cold tap water for ten minutes and removed to the stock tank of the Sheet Former where it was added to approximately 80 litres of cold tap water. The wood pulp stock was added to the water and air agitation from a ring at the bottom of the tank was begun. To this was added 1160 grams of a 1% by weight solution of Aqualon WSP M-1017 (90 parts per million for the 180 litre total volume of the stock). When foaming was observed in the stock tank, 1.5 ml of Foam Master 122 (defoamer) was added and the foaming subsided.

In the same valley beater containing approximately 10 litres of cold tap water, 460 grams of the 1% solution of Aqualon were added (200 parts per million for 23 litres), mixing was begun and foam developed. Ten drops of Foam Master 122 were added and the foam disappeared. Then 245 grams of the rayon were added slowly. Cold tap water was also added to make up 23 litres of water. This mixture was beat for fifteen minutes and then removed to the stock tank of the Sheet Former.

After the rayon stock from the beater was added to the stock tank, cold tap water was added to make up the total volume of water to 180 litres. The temperature of the mixture in the stock tank was 14°C or 57°F.

On the Sheet Former program, fresh water addition was 10 seconds; white water addition 7 seconds; stock addition 8 seconds; agitation time, 30 seconds; and settling time was 5 seconds. The average drainage time for each sheet was 10.1 seconds.

In the Pressing/Drying section, the press pressure was set at 13.79 kPa (20 psi) and the felt tension was set at 13.79 kPa (20 psi).

The physical properties of the handsheet are summarised in Table II.

**TABLE II**

| Physical Properties of Non-woven Webs | | | | |
|---|---|---|---|---|
| | | EXAMPLE 1 | EXAMPLE 2 | EXAMPLE 3 |
| Basis Weight | | | | |
| lb/3000 ft² | | 33.4 | 39.9 | 32.1 |
| g/m² | | 54.4 | 65.0 | 52.3 |

| Caliper, 3 ply | | | | |
|---|---|---|---|---|
| mils | | 58.8 | 44 | 32.8 |
| mm | | 1.49 | 1.11 | 0.83 |

| Dry Strip Tensile | | | | |
|---|---|---|---|---|
| g/3-inches | MD | 1224 | 3430 | 2034 |
| | CD | 887 | 2380 | - |
| g/cm | MD | 160 | 450 | 267 |
| | CD | 116 | 312 | - |

| Elmendorf Tear, | | | | |
|---|---|---|---|---|
| grams | MD | 54.2 | - | 57 |
| | CD | 78.8 | - | - |

| Frazier Air Permeability* | | | | |
|---|---|---|---|---|
| ft³/min/ft² | | 199.2 | 84.3 | 105.9 |
| 1/min/cm² | | 6.07 | 2.57 | 3.23 |

| | | | | |
|---|---|---|---|---|
| * 0.5 inch water Δ P (12.7 kg/m²) | | | | |

## Claims

1. A method for the preparation of a fibrous web comprising textile length fibres which comprises forming a fibre furnish by dispersion of said fibres in an unfoamed carrier medium consisting essentially of water and an associative thickener, said thickener content in the fiber furnish lying in the range of from 0.45 grams to 22.0 grams per kilogram (from 1 to 50 pounds per ton) of fiber based on the dry weight of the fibers, characterised in that the associative thickener comprises an ethylene oxide based urethane block copolymer or a hydroxyethyl cellulose ether having a C₁₀ to C₂₄ alkyl side chain, and supplying unfoamed fibre furnish at a consistency in the range of 0.05 to 0.5 weight percent fibres to the wire of a paper-making machine for forming a fibrous web.

2. A method as claimed in claim 1, characterised in that the associative thickener is a nonionic ethylene oxide based urethane block copolymer.

3. A method as claimed in claim 1, characterised in that the associative thickener is a nonionic hydroxyethyl cellulose ether having a long alkyl side chain and in that the textile length fibres are hydrophilic fibres.

4. A method as defined in claim 1, 2 or 3, characterised in that the thickener content in the fibre furnish is in a range of from 1.35 to 4.4g per kg (from 3. to 10 pounds per ton) of fibre based on the dry weight of the fibres.

5. A method as claimed in any one of the preceding claims, characterised in that the active associative thickener concentration in the liquid phase of the fibre furnish is in a range of from 25 to 120 ppm.

6. A method as claimed in any one of claims 1 to 5, characterised in that said web is composed exclusively of textile length fibres.

7. A method as claimed in any one of claims 1 to 5, characterised in that said web is composed of a mixture of cellulosic fibres and textile length fibres.

8. A. method as claimed in claim 7, characterised in that said textile length fibres are synthetic fibres.

9. A method as claimed in claim 7 or 8, characterised in that the ratio of textile length fibres to cellulose fibres is in a range of from 0.5 to 1.

10. A method as claimed in any one of claims 1 to 5 characterised in that said web comprises a mixture of cellulosic fibres and staple length synthetic textile fibers.

11. A method as claimed in claim 10, characterised in that said fibers are dispersed in water on a conventional paper-making machine.

12. A method as claimed in any one of the preceding claims, characterised in that said associative thickener has a molecular weight in the range from 10,000 to 200,000.

13. A method as claimed in any one of the preceding claims, characterised in that said textile length fibers have a length-to-diameter ratio in the range of from 300 to 3000.

14. A fibrous web produced by a method as claimed in claim 13, characterised by said web having 10 to 100 parts by weight of said textile length fibers interspersed with from 90 to 0 parts by weight wood pulp.

## Patentansprüche

1. Verfahren zum Herstellen einer Faserbahn, die Fasern textiler Länge enthält, wobei das Verfahren aufweist: Bilden eines Faserstoffeintrags durch Dispergieren der Fasern in einem ungeschäumten Trägermedium, das im wesentlichen aus Wasser und einem Assoziationsverdicker besteht, wobei der Anteil des Assoziationsverdickers in dem Faserstoffeintrag in dem Bereich von 0,45 bis 22,0 g je kg (von 1 bis 50 lbs/ton) Fasern , bezogen auf das Trockengewicht der Fasern, liegt, dadurch gekennzeichnet, daß der Assoziationsverdicker ein Urethan-Blockcopolymer auf Ethylenoxid-Basis oder ein Hydroxyethyl-Celluloseether mit einer C₁₀- bis C₂₄-Alkylseitenkette aufweist, und daß ungeschäumter Faserstoffeintrag mit einer Konsistenz im Bereich von 0,05 bis 0,5 Gew.-% Fasern auf das Sieb einer Papiermaschine zugeführt wird, um eine Faserbahn zu bilden.

2. Verfahren nach Anspruch 1, dadurch gekennzeichnet, daß der Assoziationsverdicker ein nichtionisches Urethan-Blockcopolymer auf Ethylenoxid-Basis ist.

3. Verfahren nach Anspruch 1, dadurch gekennzeichnet, daß der Assoziationsverdicker ein nichtionischer Hydroxyethyl-Celluloseether ist, der eine lange Alkylseitenkette hat, und daß die Fasern textiler Länge hydrophile Fasern sind.

4. Verfahren nach Anspruch 1, 2 oder 3, dadurch gekennzeichnet, daß der Verdickeranteil in dem Faserstoffeintrag in einem Bereich von 1,35 bis 4,4 g je kg (von 3 bis 10 lbs/ton) Fasern, bezogen auf das Trockengewicht der Fasern, liegt.

5. Verfahren nach einem der vorhergehenden Ansprüche, dadurch gekennzeichnet, daß die wirksame Assoziationsverdicker-Konzentration in der Flüssigphase des Faserstoffeintrags in einem Bereich von 25 bis 120 ppm liegt.

6. Verfahren nach einem der Ansprüche 1 bis 5, dadurch gekennzeichnet, daß die Bahn ausschließlich aus Fasern textiler Länge besteht.

7. Verfahren nach einem der Ansprüche 1 bis 5, dadurch gekennzeichnet, daß die Bahn aus einem Gemisch aus Cellulosefasern und Fasern textiler Länge besteht.

8. Verfahren nach Anspruch 7, dadurch gekennzeichnet, daR die Fasern textiler Länge synthetische Fasern sind.

9. Verfahren nach Anspruch 7 oder 8, dadurch gekennzeichnet, daß das Verhältnis von Fasern textiler Länge zu Cellulosefasern in einem Bereich von 0,5 bis 1 liegt.

10. Verfahren nach einem der Ansprüche 1 bis 5, dadurch gekennzeichnet, daß die Bahn ein Gemisch aus Cellulosefasern und synthetischen textilen Stapellängefasern ist.

11. Verfahren nach Anspruch 10, dadurch gekennzeichnet, daß die Fasern in Wasser auf einer herkömmlichen Papiermaschine dispergiert werden.

12. Verfahren nach einem der vorhergehenden Ansprüche, dadurch gekennzeichnet, daß der Assoziationsverdicker ein Molekulargewicht im Bereich von 10.000 bis 200.000 hat.

13. Verfahren nach einem der vorhergehenden Ansprüche, dadurch gekennzeichnet, daß die Fasern textiler Länge ein Länge/Durchmesser-Verhältnis im Bereich von 300 bis 3000 haben.

14. Faserbahn, die mit einem Verfahren nach Anspruch 13 hergestellt ist, dadurch gekennzeichnet, daß die Bahn 10 bis 100 Gewichtsteile der Fasern textiler Länge versetzt mit 90 bis 0 Gewichtsteilen Holzpulpe hat.

## Revendications

1. Procédé de préparation d'une nappe fibreuse comprenant des fibres textiles longues, selon lequel on forme une matière première fibreuse en dispersant ces fibres dans un milieu formant véhicule non moussé, consistant essentiellement en eau et en un épaississant associatif, la teneur en épaississant dans la matière première fibreuse étant de 0,45 g à 22,0 g/kg (de 1 à 50 livres par tonne) de fibres par rapport au poids à sec des fibres, caractérisé en ce que l'épaississant associatif comprend un copolymère séquencé d'uréthanne dérivé d'oxyde d'éthylène ou un éther d'hydroxyéthylcellulose à chaîne latérale alkyle en C₁₀ à C₂₄, et on fournit l'a matière première fibreuse non moussé selon une consistance de 0,05 à 0,5 % en poids de fibres, à la toile métallique d'une machine de fabrication de papier afin de former une nappe fibreuse.

2. Procède selon la revendication 1, caractérisé en ce que l'épaississant associatif est un copolymère séquencé d'uréthanne dérivé d'oxyde d'éthylène.

3. Procède selon la revendication 1, caractérisé en ce que l'épaississant associatif est un éther d'hydroxyéthylcellulose non ionique à longue chaîne alkyle latérale, et en ce que les fibres textiles longues sont des fibres hydrophiles.

4. Procédé selon la revendication 1, 2 ou 3, caractérisé en ce que la teneur en épaississant dans la matière première fibreuse, est de 1,35 à 4,4 g/kg (de 3 à 10 livres par tonne) de fibres par rapport au poids sec des fibres.

5. Procède selon l'une quelconque des revendications précédentes, caractérisé en ce que la concentration en épaississant associatif actif dans la phase liquide de la matière première fibreuse, est de 25 à 120 ppm.

6. Procédé selon l'une quelconque des revendications 1 à 5, caractérisé en ce que la nappe comprend exclusivement des fibres textiles longues.

7. Procédé selon l'une quelconque des revendications 1 à 5, caractérisé en ce que la nappe comprend un mélange de fibres cellulosiques et de longues fibres textiles.

8. Procédé selon la revendication 7, caractérisé en ce que les longues fibres textiles sont des fibres synthétiques.

9. Procédé selon la revendication 7 ou 8, caractérisé en ce que le rapport des longues fibres textiles aux fibres cellulosiques est de 0,5 à 1.

10. Procédé selon l'une quelconque des revendications 1 à 5, caractérisé en ce que la nappe comprend un mélange de fibres cellulosiques et de fibres textiles synthétiques longues discontinues.

11. Procédé selon la revendication 10, caractérisé en ce que les fibres sont dispersées dans de l'eau à l'intérieur d'une machine de fabrication de papier classique.

12. Procédé selon l'une quelconque des revendications précédentes, caractérisé en ce que l'épaississant associatif a un poids moléculaire de 10 000 à 200 000.

13. Procédé selon l'une quelconque des revendications précédentes, caractérisé en ce que les fibres textiles longues ont un rapport de la longueur au diamètre de 300 à 3000.

14. Nappe fibreuse produite selon un procédé revendiqué dans la revendication 13, caractérisée en ce que cette nappe comporte de 10 à 100 parties en poids desdites fibres textiles longues entremêlées avec de 90 à 0 parties en poids de pâte de bois.
